

## UNITED STATES PATENT OFFICE

HENRY DREYFUS, OF LONDON, ENGLAND

## TREATMENT OF CELLULOSIC MATERIALS AND TO THE PRODUCTION OF CELLULOSE ESTERS AND CELLULOSE ESTER PRODUCTS THEREFROM

No Drawing. Application filed December 24, 1928, Serial No. 328,306, and in Great Britain January 14, 1928.

This invention relates to the treatment of cellulosic materials for the purpose of rendering them more reactive for esterification and especially acetylation and also to the 5 production of cellulose acetates or other cellulose esters from the materials so treated.

I have now found that cellulosic materials may be rendered more reactive towards acetylation or other esterification by a treatment 10 with hydrochloric, hydrobromic or hydriodic acid or with mixtures of such hydrohalide acids or with mixtures of such hydrohalide acids with organic acids, more especially lower aliphatic acids such as formic or acetic 15 acid.

The quantity of hydrohalide acid used in the pretreatment should not exceed one half the weight of the cellulose and should preferably not be less than 2% thereof and is most 20 advantageously in the neighbourhood of 5-10% (corresponding to about 15-30% of commercial acid in the case of hydrochloric acid), though very good results are obtainable with quantities of 15-20% or even 30% on 25 the weight of the cellulose.

The hydrohalide acid may, if desired, be employed as a gas but is preferably dissolved in or diluted with a liquid, for example water. Alternately, or in addition, the hydrohalide 30 acid may be mixed or dissolved in an organic acid, particularly formic or acetic acid. Here again the hydrochloric acid or other hydrohalide acid is preferably dissolved in water and applied together with the formic, 35 acetic or other acid. The use of acetic acid in conjunction with the hydrohalide acid offers particular advantages in that it can be employed in a subsequent acetylation of the pretreated cellulose. For example the cellulose 40 may be pretreated with hydrochloric acid mixed with acetic acid in any desired quantity up to that required in the subsequent acetylation and, after the pretreatment, a catalyst may be added together with acetic anhydride 45 and if required, further acetic acid and the acetylation carried out directly.

As initial materials cotton (in either the mercerized or the non-mercerized form) or other celluloses or near conversion products 50 thereof or other cellulosic materials may be

employed. The cellulosic material used may contain the usual amount of moisture, for example, 4% to 6% or 8%, or may be freed from moisture by drying. Wood pulps, from which the lignin, pentosan, resin and like constituents have been substantially removed, 55 for example sulphite pulp, soda pulp, or sulphate pulp may be employed, but in the case of such materials the pretreatment processes of the present invention are preferably combined with and follow an alkaline purifying treatment. In such a method of treatment the wood pulp or the like is first subjected to an alkaline purifying treatment in the manner described in my U. S. Patent No. 1,711,110 60 dated April 30, 1929, for example with caustic alkali of low concentration, such as 3% or under, with heating or boiling, or with caustic alkali of higher concentration, such as 5-10% or more, in the cold or with only slight 65 heating, and then subjected to hydrohalide acid treatment in substitution for the organic acid treatment of the said U. S. Patent No. 1,711,110 dated April 30, 1929.

In conducting the pretreatment with hydrohalide acids in the liquid form, the acids may be distributed evenly over the cellulosic material, for instance by spraying the cellulose in a drum or mixer, the cellulosic material being turned from time to time if necessary to ensure uniform impregnation. The 75 cellulosic material is then allowed to stand until a product capable of rapid esterification is obtained, for example for 1 to 2 up to 12 or 24 hours or more. The pretreatment may 80 be carried out with gaseous hydrohalide acids, preferably in admixture with vapours of organic acids.

The time required for the pretreatment varies with the nature of the cellulosic material, the concentration of the pretreating agent or agents, the temperature at which the cellulosic material is maintained, and the degree of reactivity required in the product. The treatment is preferably carried out at ordinary temperatures but may, if desired, be 90 accelerated by the use of somewhat increased temperatures.

The use of higher temperatures which 95 would result in disintegration of the cellulose 100

must be avoided. Similarly large quantities of hydrohalide acid must not be used. The quantity of hydrohalide acid should not exceed 50% (calculated as hydrogen halide) of the weight of the cellulose and is preferably much less than this.

The subsequent acetylation or esterification of the cellulosic materials thus treated may be carried out by any suitable process. If 10 the hydrohalide acid used in the pretreatment be not required or be required in smaller quantity in the acetylation or esterification, it may be wholly or partially neutralized, for example by addition of sodium or other acetate. Formic acid when employed in conjunction with hydrohalide acid in the pretreatment should, except when used in comparatively small quantities (see prior U. S. application S. No. 162,218 dated 19th January 1927), be removed or substantially removed before acetylation with acetic anhydride as it reacts therewith. Any acetic acid employed in the pretreatment may remain in the cellulosic material to act as part of the 25 esterifying mixture in the subsequent esterification.

The process of pretreatment according to the present invention offers the greatest advantages when the subsequent acetylation 30 or esterification is carried out according to the processes described in my prior U. S. application S. No. 301,927 dated 24th August 1928, 321,750 dated 24th November 1928 and 321,751 dated 24th November, 1928. 35 These specifications describe acetylation or esterification in presence of (a) halides of iron, manganese, cobalt, nickel or copper in conjunction with a hydrohalide acid, each being present in a quantity not less than 2% 40 on the cellulose; (b) ferric halide without hydrohalide acid; and (c) stannic halide with or without hydrohalide acid.

In acetylating or esterifying according to the processes described in my said prior applications, the hydrohalide acid used in the pretreatment need not be removed and it is therefore possible to proceed directly from the pretreatment to the esterification of the cellulose. If the hydrohalide acid be required in the acetylation or esterification the metal or other halide to be used in conjunction therewith, together with any additional hydrohalide acid if required, may be added to the pretreated cellulose separately or together 50 with the acetylating or esterifying agent. When the acetylating or esterifying agent is to be added together with the halide salt, the latter may, if desired, be formed in situ in the acetylating or esterifying mixture. Instead of adding the halide salt as such, a substance such as ferric oxide or ferric acetate 55 may be used so as to form the required halide salt by interaction with part of the hydrohalide acid already in the cellulose. If no hydrohalide acid be required in the esterifica-

tion, the residual acid in the cellulose after the pretreatment may be employed to form the required halide catalysts in situ. For example by adding ferric oxide or ferric acetate or the like to a cellulosic material pretreated with hydrochloric acid, ferric chloride for use as a catalyst may be formed within the cellulosic material. It is to be noted however that even in the case of acetylating or esterifying according to the processes of these prior applications, the present invention is not limited to the non removal of the hydrohalide acid.

The acetylation or other esterification may be conducted in presence of a solvent for 80 the cellulose ester produced or in presence of a non-solvent diluent or in the absence of solvents or diluents by employing a vaporous esterifying agent.

The following examples illustrate the processes of pretreatment according to the present invention and the preferred methods of subsequent esterification, but they are not to be considered as limiting the invention in any way.

#### Example 1

100 parts of cotton cellulose are sprayed with 15 to 30 parts of concentrated hydrochloric acid (about 33% strength) and allowed to stand with occasional turning for 2 to 3 hours at normal temperature. The pretreated material is then introduced in the acetylator into a mixture of 800 parts of acetic acid, 300 parts of acetic anhydride and 15 parts of ferric chloride. The acetylation is carried out in the cold with constant mixing or stirring. A clear solution of cellulose acetate of high viscosity is obtained.

#### Example 2

100 parts of cotton cellulose are sprayed with a mixture containing 15-30 parts of concentrated hydrochloric acid and 30-50 parts of acetic acid. The pretreatment is carried out in the cold with occasional stirring for 2 to 6 hours. The pretreated material is then introduced into a mixture of 600 parts of acetic anhydride, 550 parts of acetic acid and 10 to 15 parts of ferric chloride in an acetylator. The reaction is conducted at normal temperature with constant mixing or stirring and is complete in from 5 to 20 hours, a clear solution being obtained.

#### Example 3

100 parts of cotton cellulose are introduced in an acetylator into a mixture of 600 parts of acetic acid and 30 parts of hydrochloric acid and allowed to stand with stirring for 3 to 7 hours. Thereafter there are added 10 parts of stannic chloride and 600 parts of acetic anhydride and the mass is constantly stirred throughout the reaction which is car-

ried out at about normal temperature. The acetylation proceeds smoothly and a clear solution is obtained.

The cellulose acetates or cellulose esters obtained may be used in their esterification solutions (more particularly when the esterification is carried out according to the prior applications referred to) or in solutions of the primary esterification products for the production of artificial silks, films etc. or they may be subjected to secondary treatments or reactions for the purpose of changing their solubilities i. e. the so-called ripening. The secondary treatments or ripening may be carried out in the primary esterification solutions or suspensions, preferably without neutralizing the hydrochloric or other hydrohalide acid, if present, and preferably without eliminating any halide catalyst if used and after destroying if necessary any remaining anhydride by the addition of water or other anhydride destroying agents, such for instance as hydroxyl derivatives, oxy acids, for instance lactic acid, alcohols etc. If no acid catalyst be used in the esterification, hydrochloric or other hydrohalide acid may, if desired, be added to accelerate the reaction. Alternatively, the esters either precipitated from the primary esterification solutions or those obtained other than in solution may be dissolved or suspended and then subjected to the secondary treatments or ripening. The secondary treatments or reactions may be carried out with or without addition of inorganic or organic acids, acid salts or other suitable agents for promoting the secondary treatment or reaction, the treatment in any case being stopped when the required solubility has been reached. It is particularly advantageous to conduct the further treatments or reactions in the joint presence of hydrohalide acid and metal halide or other catalysts used according to the prior applications referred to, either in the primitive esterification solutions or suspensions or after separation therefrom. For the ripening or further treatments or reactions one should first destroy any remaining acetic anhydride or other esterifying anhydride that may remain in the esterification solution or suspension or in the primary ester, by adding water or other anhydride destroying agents to the esterification solution or to the solutions or suspensions of the primary ester.

While the ripening or secondary or further treatments of the primary esterification products may with advantage be conducted at ordinary or moderate temperatures, one may if desired quicken the reaction by heating up to relatively high or high temperatures even up to 80° or 100° C. or higher, but in such cases the presence of free mineral acids is preferably avoided.

The secondary or further treatments of the

primary esterification products will be stopped when the particular solubility desired is reached.

In carrying out the esterification with halide catalysts according to the methods described in my said prior applications and the secondary treatments or ripening according to the preferred methods described therein, it will be seen that very considerable advantages accrue, since a continuous series of processes is possible without any separation of reagents at intermediate stages. For example a cellulosic material may be pre-treated with 5-10% of its weight of hydrochloric acid (calculated as HCl) in aqueous solution, a quantity of ferric chloride equal to (say) 5-10% of the weight of the cellulosic material added together with acetic anhydride and acetic acid and finally, after the acetylation, a secondary reaction or ripening carried out directly in presence of the hydrochloric acid and ferric chloride.

The cellulose acetates or other esters can be employed in their primary esterification solutions in their different stages or phases of acetylation, for the production of artificial silks and the like, films, celluloid-substitutes or other thermo-plastic masses, moulding powders or articles, etc.

Further the invention permits of obtaining cellulose esters of high quality which are soluble in acetone or in very low boiling solvents, for instance methyl formate, acetaldehyde, formaldehyde etc. Also suitable high boiling solvents or plasticizing or softening agents can be readily incorporated with them or their solutions in volatile solvents and/or very low boiling solvents.

The cellulose acetates or other esters, either in their primary esterification solutions and with or without secondary treatments or ripening, or as primary or secondary esters in solution in suitable solvents, for example acetone, ethyl alcohol-acetone, methyl alcohol-acetone, or the very low boiling solvents specified above or in mixtures of such solvents, may be employed for the production of artificial silks or fibers, films etc. For either wet or dry spinning processes the esters may be employed in the form of solutions of relatively low concentration, for instance 5-8%, or of medium concentration, for example 10-20% or of high concentration containing over 20% e. g. 25-30% or more.

The term "disintegration" is employed in the specification and claims as connoting loss of structure.

What I claim and desire to secure by Letters Patent is:—

1. Process for the treatment of material consisting substantially of cellulose without substantial disintegration, comprising treating the material with up to 50% of its weight of hydrogen halide under conditions to avoid

substantial disintegration of the cellulose, whereby it is rendered more reactive to esterification.

2. Process for the treatment of material consisting substantially of cellulose without substantial disintegration, comprising treating the material with up to 50% of its weight of hydrogen chloride under such conditions to avoid substantial disintegration of the cellulose, whereby it is rendered more reactive to esterification.

3. Process for the treatment of material consisting substantially of cellulose without substantial disintegration, comprising treating the material with up to 50% of its weight of hydrogen halide in aqueous solution under such conditions to avoid substantial disintegration of the cellulose, whereby it is rendered more reactive to esterification.

4. Process for the treatment of material consisting substantially of cellulose without substantial disintegration, comprising treating the material with up to 50% of its weight of hydrogen chloride in aqueous solution under such conditions to avoid substantial disintegration of the cellulose, whereby it is rendered more reactive to esterification.

5. Process for the treatment of material consisting substantially of cellulose without substantial disintegration, comprising treating the material at normal temperature, with up to 50% of its weight of hydrogen chloride under such conditions to avoid substantial disintegration of the cellulose, whereby it is rendered more reactive to esterification.

6. Process for the treatment of material consisting substantially of cellulose without substantial disintegration, comprising treating the material at normal temperature, with up to 50% of its weight of hydrogen chloride in aqueous solution under such conditions to avoid substantial disintegration of the cellulose, whereby it is rendered more reactive to esterification.

7. Process for the treatment of material consisting substantially of cellulose without substantial disintegration, comprising treating the material with organic acid and with up to 50% of its weight of hydrogen halide under such conditions to avoid substantial disintegration of the cellulose, whereby it is rendered more reactive to esterification.

8. Process for the treatment of material consisting substantially of cellulose without substantial disintegration, comprising treating the material with acetic acid and with up to 50% of its weight of hydrogen chloride in aqueous solution under such conditions to avoid substantial disintegration of the cellulose, whereby it is rendered more reactive to esterification.

9. Process for the treatment of material consisting substantially of cellulose without substantial disintegration, comprising treating the material with up to 50% of its weight

of hydrogen halide under such conditions to avoid substantial disintegration of the cellulose, and thereafter esterifying it.

10. Process for the treatment of cellulosic material, comprising treating the material with up to 50% of its weight of hydrogen chloride without substantial disintegration and thereafter acetylating with acetic anhydride. 70

11. Process for the treatment of material consisting substantially of cellulose, comprising treating the material with up to 50% of its weight of hydrogen chloride in aqueous solution without substantial disintegration, and thereafter acetylating with acetic anhydride in presence of halide catalysts. 75

12. Process for the treatment of material consisting substantially of cellulose, comprising treating the material with acetic acid and with up to 50% of its weight of hydrogen chloride in aqueous solution without substantial disintegration and thereafter acetylating with acetic anhydride in presence of halide catalysts. 80

13. Process for the treatment of material consisting substantially of cellulose without substantial disintegration comprising treating the material with a lower fatty acid and with up to 50% of its weight of hydrogen halide at substantially normal temperatures 95 whereby it is rendered more reactive to esterification. 90

14. Process for the treatment of material consisting substantially of cellulose without substantial disintegration, comprising treating the material with acetic acid and with up to 50% of its weight of hydrogen chloride in aqueous solution at substantially normal temperatures, whereby it is rendered more reactive to esterification. 100

15. Process for the treatment of material consisting substantially of cellulose without substantial disintegration, comprising treating the material with up to 50% of its weight of hydrogen halide at substantially normal temperatures and thereafter esterifying it. 110

16. Process for the treatment of material consisting substantially of cellulose comprising treating the material with up to 50% of its weight of hydrogen chloride at substantially normal temperatures without substantial disintegration, and thereafter acetylating it with acetic anhydride. 115

17. Process for the treatment of material consisting substantially of cellulose, comprising treating the material with acetic acid and with up to 50% of its weight of hydrogen chloride in aqueous solution at substantially normal temperatures without substantial disintegration and thereafter acetylating with acetic anhydride in the presence of halide catalysts. 120

In testimony whereof I have hereunto subscribed my name.

HENRY DREYFUS. 125